

# UNITED STATES PATENT OFFICE.

GEORGE ENNIS FERGUSON, OF NEW YORK, N. Y., ASSIGNOR TO PYRENE MANUFACTURING COMPANY, A CORPORATION OF DELAWARE.

## FIREPROOFING SOLUTION.

1,261,736.

Specification of Letters Patent.

Patented Apr. 2, 1918.

No Drawing.

Application filed September 30, 1915. Serial No. 53,309.

*To all whom it may concern:*

Be it known that I, GEORGE E. FERGUSON, a citizen of the United States, residing at the city, county, and State of New York, have invented a new and useful Improvement in Fireproofing Solutions, of which the following is a specification.

This invention relates to a fire proofing solution, the object being to provide a solution with which fibrous material or fabric may be impregnated to render the same non-inflammable.

Such solutions have been used before my invention, but, so far as I am aware, the fire proofing substance in the solution is soluble in water.

The particular object and nature of this invention is to provide a fire proofing solution in which the fire retarding substance, or substances, are insoluble in water, thus rendering the fabric treated with the same, permanently fire proof.

To accomplish this result, I employ a solvent containing a volatile substance and in which fire proofing substances are dissolved, which substances are insoluble in water, and the solvent containing the dissolved substances being readily absorbed by the fabric. At the same time it is desirable to use materials which will do no damage to the fabric when absorbed.

Certain compounds which are insoluble in water are readily soluble in ammonium hydroxid. For example, copper phosphate, copper oxalate, cuprous chlorid, copper hydroxid, zinc phosphate, zinc oxid, zinc hydroxid, etc.

Examples of solvents suitable for this purpose are ammonium hydroxid, alcohols, benzin, ether, chloroform, carbon tetra chlorid or the volatile chlorinated hydrocarbons, etc. Of these solvents, the most desirable, from the standpoint of cost and capability to dissolve certain water insoluble salts, is ammonium hydroxid, consequently, this will be used as an example for explaining the action of the fire proofing solution. If, for example, zinc phosphate is dissolved in ammonium hydroxid, the quantity being determined by the use to which the fabric is to be put, a clear transparent solution is formed, which is readily absorbed by the fabric.

It was also found to be advantageous when forming the above solution, to dissolve a small quantity of zinc chlorid therein. The zinc chlorid is first precipitated as zinc hydroxid, which is soluble in an excess of the ammonium hydroxid. Fabrics submerged in this liquid will absorb the solution and when exposed to the air, particularly warm air, the ammonium hydroxid, is volatilized off and the water insoluble salts, zinc phosphate and zinc hydroxid, are left in the fabric. As these salts are insoluble in water, immersion of the fabric in water will fail to dislodge them, and the fabric thus treated will not burn, even if held in the flame of the Bunsen burner. It will carbonize but not burn.

A further advantage obtained in using ammonium hydroxid for the solvent, is that it will saponify or dissolve any oil or grease in the fabric, and after the fabric is impregnated with the salts, it will have water repellent properties, thus rendering the fabric fire and water proof.

I do not wish to be understood as limiting my invention to the specific substances herein set out as illustrative of the types of substances which may be employed, or to the specific fluids which may be used, as it is undoubtedly possible to substitute other ingredients without departing from the spirit of the invention.

What I claim is:

1. A fire proofing solution comprising a solvent containing a volatile substance, and phosphate of zinc and hydrate of zinc dissolved therein.

2. A fire proofing solution comprising ammonium hydroxid with zinc phosphate and zinc chlorid dissolved therein, the zinc chlorid being precipitated as zinc hydroxid and then dissolved in the ammonium hydroxid.

In testimony whereof, I, the said GEORGE E. FERGUSON, have signed my name to this specification in the presence of two subscribing witnesses, this 24<sup>th</sup> day of Sept. 1915.

GEORGE ENNIS FERGUSON.

Witnesses:

LEWIS J. DOOLITTLE,  
THEODORE B. T. MERKS.